

## UNITED STATES PATENT OFFICE

ISADORE M. JACOBSON, OF CHICAGO, ILLINOIS, AND STARR TRUSCOTT, OF BIRMINGHAM, OHIO

## AIRCRAFT COVERING

No Drawing.

Application filed March 5, 1926. Serial No. 92,645.

This invention relates to a gas retaining fabric for aircraft coverings using an impermeable film prepared from a mixture of cuprammonium cellulose or the like and a latex.

It is, however, to be understood that without material modification the fabric is applicable to various other uses and applications.

10 The disadvantages of a gas retaining fabric using goldbeater's skin as an impermeable membrane are well known to those skilled in the art and the present invention is intended to overcome various disadvantages incident to 15 the preparation of such skins.

It has been found that a film produced from a mixture of cuprammonium cellulose or other water soluble form of cellulose, and latex has a very high resistance to the passage of the buoyant gases. Such material can be produced either in large sheets or spread directly upon cloth in a manner similar to that by which rubber is applied.

The following will illustrate the method 25 of preparing gas impermeable fabrics from a mixture of cuprammonium cellulose and latex. Dissolve 0.29 gm. of tetramethyl thiuram disulfide in 15 cc. of hot acetone. Add this solution quickly to 400 cc. of water at 20°

30 C. This is immediately followed by the addition, with vigorous agitation, of 70 gms. of rubber latex containing 40% of solid matter. It is essential that this operation be carried out very promptly in order to prevent the coagulation of the first material added. Three 35 gms. of zinc sulfate, dissolved in 10 cc. of water, are treated with 7 cc. of ammonia water containing 29% of ammonia. The white precipitate formed at first should be completely

40 dissolved before proceeding further. This solution is then added to the latex solution above, with vigorous agitation. 250 gms. of cuprammonium cellulose are then added to the mixture and stirred until a homogeneous 45 mixture results. The cuprammonium cellulose-latex mixture prepared by the above method should be kept at a temperature not exceeding 20° C. until applied.

4 In order to prepare a gas impermeable fabric from the cuprammonium cellulose-latex

mixture, it is spread upon a balloon cloth, spreading in 8 to 15 coats, depending upon the permeability desired. Each coat is dried by the passage over its surface of a current of air, heated to 40° C. before the application 55 of the next coat. When the last coat is dry, the fabric is immersed in a 2% solution of sulfuric acid in order to dissolve the copper oxide which is deposited with the film. The fabric is then washed thoroughly with water 60 and finally immersed in a 15% solution of glycerine. The fabric is then air dried. The immersion in a solution of glycerine renders the material plastic, permitting creasing or folding without its being subjected to cracking or breaking. 65

It is thus seen that the present invention comprehends a simple and practical fabric suitable as a substitute for goldbeater's skin and well adapted to accomplish, among others, 70 the various objects and advantages herein set forth.

The invention herein described may be manufactured and used by or for the Government of the United States for governmental 75 purposes without the payment to us of any royalty thereon or therefor.

What we claim is:—

1. A fabric coated with a film of reverted cuprammonium cellulose-latex immersed in 80 glycerine whereby the fabric is rendered flexible and impermeable to gases.

2. A method of rendering a fabric flexible and impermeable to gases consisting in coating a fabric with a mixture of cuprammonium 85 cellulose-latex, bathing the coated fabric in sulfuric acid, washing to remove any reaction products, immersing in a plasticizing agent, and finally drying.

3. A fabric coated with a film of reverted 90 plasticized cuprammonium-cellulose-rubber.

Signed at Washington, District of Columbia, this 13th day of November, 1925.

ISADORE M. JACOBSON.  
STARR TRUSCOTT.

95